

Patented Feb. 12, 1935

1,990,474

# UNITED STATES PATENT OFFICE

1,990,474

## OIL ACID VARNISH AND PRODUCT COATED THEREWITH

Alfonso M. Alvarado, Wilmington, Del., assignor to E. I. du Pont de Nemours & Company, Wilmington, Del., a corporation of Delaware

No Drawing. Application March 7, 1931,  
Serial No. 520,998

11 Claims. (Cl. 91—70)

This invention relates to the production of coating compositions and products coated therewith, and more particularly it relates to artificial leather finished with an improved top coat. Still more specifically the invention relates to compositions suitable for finishing rubber coated fabrics such as are used for automobile tops, rubber upholstery, etc., and to the improved products resulting from finishing such fabrics with the coating compositions described herein. This invention has as an object the production of coating compositions particularly suitable as finishes or top coats for fabrics in the manufacture of artificial leather. A further object is the production of fabrics, particularly rubber coated fabrics, provided with a top coat having a high gloss, a deep black color, freedom from blueness, excellent durability, and good retention of gloss even after prolonged exposure to the weather. These objects, in their broader aspects, are accomplished by the manufacture of varnishes from asphalt and fatty acids and application of these varnishes, with subsequent baking or drying, to the article to be finished. These asphaltic varnishes, which are particularly advantageous for the finishing of rubber coated fabrics in the manufacture of automobile top material and artificial leather in general, are conveniently made by blending a solution of asphalt with a free fatty acid derived from drying, semi-drying, or non-drying oils, with or without the addition of the usual varnish driers. It is preferable, however, to add organic compounds of metals, which compounds function not only as driers but also as blending agents between the oil acids and the asphalt. Organic compounds of iron are particularly valuable as blending agents. If desired, the oil acids may be heat-treated or blown (either in the presence or absence of organic salts of metals) prior to blending with the asphalt. In general, I prefer to heat-treat in the presence of an organic salt of a metal, especially an iron organic compound. Suitable varnishes comprising free fatty acids and asphalt, and the method for their preparation, are indicated in the following fourteen examples:

### Example I

|                           | Parts<br>by weight |
|---------------------------|--------------------|
| Petroleum residue asphalt | 100.00             |
| Solvent naphtha           | 100.00             |
| Turpentine substitute     | 40.00              |
| China wood oil acids      | 40.00              |
| Total                     | 280.00             |

The asphalt is heated to 500° F., allowed to cool to 425° F., an equal weight of solvent naphtha is added, and the mixture is stirred until the asphalt is completely dissolved. To this solution

is added 80 parts by weight of a 50% of China wood oil acids in turpentine substitute.

### Example II

|                                         | Parts<br>by weight |
|-----------------------------------------|--------------------|
| Petroleum residue asphalt               | 100.00             |
| Solvent naphtha                         | 100.48             |
| China wood oil acids                    | 20.00              |
| Turpentine                              | 20.00              |
| Cobalt linoleate (containing 5.80% Co.) | 0.17               |
| Total                                   | 240.65             |

The asphalt is heated to 500° F., allowed to cool to 425° F., an equal weight of solvent naphtha is added, and the mixture is stirred until the asphalt is completely dissolved. To this solution is added 40 parts by weight of a 50% solution of China wood oil acids in turpentine and 0.65 parts by weight of a cobalt linoleate solution in solvent naphtha, said solution containing 1.45% cobalt.

### Example III

|                                | Parts<br>by weight |
|--------------------------------|--------------------|
| Petroleum residue asphalt      | 100.00             |
| Solvent naphtha                | 110.80             |
| Linseed oil acids              | 160.00             |
| Turpentine                     | 160.00             |
| Lead resinate (10% Pb.)        | 2.40               |
| Manganese resinate (6.63% Mn.) | 1.20               |
| Total                          | 534.40             |

The asphalt is heated to 500° F., allowed to cool to 425° F., an equal weight of solvent naphtha is added, and the mixture is stirred until the asphalt is completely dissolved. To this solution is added 320 parts by weight of a 50% solution of linseed oil acids in turpentine, 9.6 parts by weight of a lead resinate drier solution, and 4.8 parts by weight of a manganese resinate drier solution, said solutions containing 2.50% lead and 1.66% manganese, respectively.

### Example IV

|                                | Parts<br>by weight |
|--------------------------------|--------------------|
| Gilsonite                      | 100.00             |
| Solvent naphtha                | 103.70             |
| Castor oil acids               | 40.00              |
| Turpentine                     | 40.00              |
| Lead resinate (10% Pb.)        | 0.60               |
| Manganese resinate (6.63% Mn.) | 0.30               |
| Total                          | 283.60             |

The gilsonite is heated to 500° F., allowed to cool to 425° F., an equal weight of solvent naphtha is added, and the mixture is stirred until the asphalt is completely dissolved. To this solution

is added 80 parts by weight of a 50% solution of castor oil acids in turpentine, 2.4 parts by weight of a lead resinate solution in solvent naphtha, and 1.2 parts by weight of a manganese 5 resinate drier solution in solvent naphtha, said solutions containing 2.50% lead and 1.66% manganese, respectively.

The asphalt is heated to 500° F., allowed to cool to 425° F., an equal weight of solvent naphtha is added, and the mixture is stirred until the asphalt is completely dissolved. To this solution is added 320 parts by weight of a 50% solution of cottonseed oil acids in turpentine and 58.8 parts by weight of a solution of iron linoleate in solvent naphtha, said solution containing 2.73% iron. 5

*Example V*

|                              | Parts<br>by weight |  |
|------------------------------|--------------------|--|
| 10 Petroleum residue asphalt | 100.00             |  |
| Solvent naphtha              | 153.63             |  |
| Oleic acid                   | 200.00             |  |
| 15 Turpentine                | 200.00             |  |
| Iron resinate                | 28.35              |  |
| <b>Total</b>                 | <b>681.98</b>      |  |

The asphalt is heated to 500° F., allowed to cool to 425° F., an equal weight of solvent naphtha is added, and the mixture is stirred until the asphalt is completely dissolved. To this solution is added 400 parts by weight of a 50% solution of oleic acid in turpentine and 82 parts by weight of a solution of iron resinate in solvent naphtha, said solution containing 2.44% iron. 25

*Example VI*

|                              | Parts<br>by weight |  |
|------------------------------|--------------------|--|
| 30 Petroleum residue asphalt | 100.00             |  |
| Solvent naphtha              | 130.00             |  |
| China wood oil acids         | 240.00             |  |
| Turpentine                   | 240.00             |  |
| 35 Iron oleate               | 30.00              |  |
| <b>Total</b>                 | <b>740.00</b>      |  |

The asphalt is heated to 500° F., allowed to cool to 425° F., an equal weight of solvent naphtha is added, and the mixture is stirred until the asphalt is completely dissolved. To this solution is added 480 parts by weight of a 50% solution of China wood oil acids in turpentine and 60 parts by weight of a solution of iron oleate in solvent naphtha, said solution containing 4% iron. 45

*Example VII*

|                              | Parts<br>by weight |  |
|------------------------------|--------------------|--|
| 50 Petroleum residue asphalt | 100.00             |  |
| Solvent naphtha              | 110.93             |  |
| Soya bean oil acids          | 40.00              |  |
| Turpentine                   | 40.00              |  |
| Iron resinate                | 5.47               |  |
| <b>55 Total</b>              | <b>296.40</b>      |  |

The asphalt is heated to 500° F., allowed to cool to 425° F., an equal weight of solvent naphtha is added, and the mixture is stirred until the asphalt is completely dissolved. To this solution is added 80 parts by weight of a 50% solution of soya bean oil acids in turpentine and 16.4 parts by weight of a solution of iron resinate in solvent naphtha, said solution containing 2.44% iron. 60 65

*Example VIII*

|                           | Parts<br>by weight |  |
|---------------------------|--------------------|--|
| Petroleum residue asphalt | 100.00             |  |
| 70 Solvent naphtha        | 129.40             |  |
| Cottonseed oil acids      | 160.00             |  |
| Turpentine                | 160.00             |  |
| Iron linoleate            | 29.40              |  |
| <b>75 Total</b>           | <b>578.80</b>      |  |

*Example IX*

|                   | Parts<br>by weight |    |
|-------------------|--------------------|----|
| Gilsonite         | 100.00             |    |
| Solvent naphtha   | 102.50             |    |
| Coconut oil acids | 20.00              | 15 |
| Turpentine        | 20.00              |    |
| Iron oleate       | 2.50               |    |
| <b>Total</b>      | <b>245.00</b>      |    |

The gilsonite is heated to 500° F., allowed to cool to 425° F., an equal weight of solvent naphtha is added, and the mixture is stirred until the gilsonite is completely dissolved. To this solution is added 40 parts by weight of a 50% solution of coconut oil acids in turpentine and 5 parts by weight of a solution of iron oleate in solvent naphtha, said solution containing 4% iron. 20 25

*Example X*

|                             | Parts<br>by weight |    |
|-----------------------------|--------------------|----|
| Petroleum residue asphalt   | 100.00             |    |
| Solvent naphtha             | 100.00             |    |
| Bodied China wood oil acids | 55.17              | 35 |
| Turpentine                  | 60.00              |    |
| Iron laurate                | 4.83               |    |
| <b>Total</b>                | <b>320.00</b>      |    |

The asphalt is heated to 500° F., allowed to cool to 425° F., an equal weight of solvent naphtha is added, and the mixture is stirred until the asphalt is completely dissolved. To this solution is added 120 parts by weight of a 50% turpentine solution of China wood oil acids bodied with iron laurate. (By iron laurate is meant the reaction product of iron salts with coconut oil acids). The mixture of China wood oil acids with iron laurate is prepared from the following ingredients as indicated below: 40 45

|                                       | Parts<br>by weight |    |
|---------------------------------------|--------------------|----|
| China wood oil acids                  | 91.95              |    |
| Iron laurate (containing 11.43% iron) | 8.05               | 55 |

**Total** 100.00

The China wood oil acids are heated to 385° F. and the iron laurate is added slowly and with constant stirring. The mixture is then heated to 425° F. in the course of one hour and kept at this temperature for two hours. 60

*Example XI*

|                           | Parts<br>by weight |    |
|---------------------------|--------------------|----|
| Petroleum residue asphalt | 100.00             |    |
| Solvent naphtha           | 100.00             |    |
| Turpentine                | 160.00             |    |
| Bodied linseed oil acids  | 140.72             | 70 |
| Iron resinate             | 19.28              |    |
| <b>Total</b>              | <b>520.00</b>      |    |

The asphalt is heated to 500° F., allowed to cool to 425° F., an equal weight of solvent naphtha is 75

added, and the mixture is stirred until the asphalt is completely dissolved. To this solution is added 320 parts by weight of a 50% turpentine solution of linseed oil acids bodied with iron resinate, prepared from the following ingredients as indicated below:

|                                         | Parts<br>by weight |
|-----------------------------------------|--------------------|
| Linseed oil acids                       | 87.95              |
| 10 Iron resinate (containing 7.3% iron) | 12.05              |
| Total                                   | 100.00             |

The linseed oil acids are heated to 450° F. and the iron resinate is added slowly and with constant stirring. The oil acids are then heated to 525° F. in the course of one hour and kept at this temperature for two hours.

*Example XII*

|                           | Parts<br>by weight |
|---------------------------|--------------------|
| Petroleum residue asphalt | 100.00             |
| Solvent naphtha           | 121.90             |
| China wood oil acids      | 40.00              |
| 25 Linseed oil acids      | 40.00              |
| Iron resinate             | 10.90              |
| Total                     | 312.80             |

The asphalt is heated to 500° F., allowed to cool to 425° F., an equal weight of solvent naphtha is added, and the mixture is stirred until the asphalt is completely dissolved. To this solution is added 160 parts by weight of a 50% solution of a 1:1 mixture of China wood oil acids and linseed oil acids in turpentine and 32.8 parts by weight of a solution of iron resinate in solvent naphtha, said solution containing 2.44% iron.

The following are examples of formulae containing pigments. The ingredients are compounded in accordance with the method set forth in the previous examples.

*Example XIII*

|                           | Parts<br>by weight |
|---------------------------|--------------------|
| Petroleum residue asphalt | 100.00             |
| China wood oil acids      | 160.00             |
| Carbon black              | 26.00              |
| 50 Solvent naphtha        | 364.00             |
| Iron resinate             | 21.84              |
| Total                     | 671.84             |

*Example XIV*

|                           | Parts<br>by weight |
|---------------------------|--------------------|
| Petroleum residue asphalt | 100.00             |
| China wood oil acids      | 320.00             |
| 60 Carbon black           | 69.32              |
| Solvent naphtha           | 537.23             |
| Iron resinate             | 43.67              |
| Total                     | 1070.22            |

65 Certain oil acids, such as China wood oil acids, are remarkable in their compatibility characteristics with asphaltic materials, especially with petroleum residue asphalts, which are generally difficultly compatible with drying oils. This remarkable compatibility of oil acids with asphalts is shown by the fact that 100 gallon varnishes can be successfully prepared with petroleum residue asphalts and either China wood oil acids or mixtures of equal proportions of China wood oil acids and either oleic acid or linseed oil acids.

In spite of this exceptional compatibility, I usually do not prefer to use asphalt varnishes above 20 gallons in oil acid length when no pigments are used. When pigments are used, however, forty gallon varnishes can be employed with excellent results. To a certain extent, of course, the preferred gallon lengths depend upon the kind of oil acids used. Thus, castor oil acid varnishes of longer gallon length than 5 gallons cannot be satisfactorily prepared, whereas with China wood oil acids 100 gallon varnishes can be prepared which are satisfactorily compatible.

A "gallon" oil length, as used in the varnish trade, designates a gallon of oil per 100 pounds of gum. By weight, this is generally about 8 15 pounds of oil to 100 pounds of gum. The terms "gallon" or "gallon length" or "gallon oil acid length", as used herein, designates 8 pounds of oil acids per 100 pounds of asphalt or mixture of asphalt with resin, such as ester gum, limed rosin, 20 glycerol-phthalate resin containing rosin in combined form, and oil soluble phenol-formaldehyde resin. For example, a 5 gallon asphalt-oil acid varnish contains approximately 40 pounds of oil acids to 100 pounds of asphalt.

Instead of blending solutions of asphalt and free fatty acids, as in the examples, the asphalts may be blended with the oil acids at elevated temperatures, the blend diluted with the required amount of solvent, and the drier or iron organic compound added to the mixture.

It is desirable, in some instances, to use combinations of asphalts with mixtures of oil acids. When mixtures of oil acids are used, it is sometimes desirable to heat-treat or to blow one of the oil acids or the mixture of oil acids prior to blending with the asphalts. Substantial improvements may sometimes be obtained by using mixture of oils with oil acids in the preparation of these varnishes. In order to increase the 40 durability and to improve the drying qualities of these varnishes, pigments may be incorporated therewith. When pigments are used, however, it is preferred to use pigments which will not react with the oil acids. In varnishes designed for use under severe conditions of weathering, I prefer to use a steam refined asphalt in preference to asphalts refined by other methods, such as by blowing with air. The term "steam refined petroleum residue asphalt varnish", as used herein, is intended to designate coating compositions in which the principal film-forming constituents are steam refined petroleum residue asphalts and drying oil acids. However, in some cases it is advantageous to use air blown asphalts, gilsonite, or other bitumens in place of steam refined petroleum residue asphalts.

When other asphalts or bitumens are used, however, a lower order of durability is generally obtained than when steam refined petroleum residue asphalts are used. Whereas I have mentioned ordinary varnish driers and iron organic compounds as desirable ingredients of these varnishes, it will be apparent that inorganic salts of cobalt, lead, manganese, iron, or other metals, not ordinarily used as varnish driers, may be added and caused to react with the oil acid components of the varnish, thus forming compounds effective as driers or blending agents.

The process of the present invention finds wide 70 application in the manufacture of rubber coated fabric for automobile top material. In the one-coat system, which is the simplest form of my invention, the coat of asphalt-oil acid varnish is applied over the uncured rubber and then sub-

jected to heating at a suitable temperature and for a sufficient time to vulcanize the rubber and to thoroughly fuse the varnish film. By this treatment I obtain on the surface of the goods 5 a smooth, continuous film which is substantially inert and which remains for a long time unaffected by sunlight. The temperature and time of cure depend on the rubber compound, and especially on the kind and quantity of vulcanizing agent used. As a rule, the temperature will lie between 240° F. and 275° F., and the time of cure will be from 30 minutes to 3 hours.

When using my two-coat system, I first apply to the uncured rubber an intermediate coat of 10 varnish which is preferably more flexible than the asphalt-oil acid varnish used as the final coat. Excellent results are obtained, however, through application of two coats of the asphalt-oil acid varnish. The intermediate coat may be 15 air-dried, if desired, that is, dried at room temperature, but it is more advantageous from the cost standpoint to use a "force-dry", that is, dry at an elevated temperature but below the vulcanizing temperature of the rubber. Thus, I 20 usually dry the first coat varnish by heating it up to 250° F. to 270° F. in one hour, after which I apply the final varnish coat and finish by baking at a temperature of about 240° F. to 275° F. for such time as is required to complete the vulcanization of the rubber.

The following is an example of a suitable undercoat varnish for the above varnishes:

*Example XV*

|                                 | Parts by<br>weight |
|---------------------------------|--------------------|
| Carbon black                    | 2.5                |
| Bodied China wood oil and drier | 20.0               |
| Bodied linseed oil and drier    | 20.0               |
| Turpentine substitute           | 54.0               |
| Petroleum residue asphalt       | 3.5                |
| <br>Total                       | <br>100.0          |

In some cases it is advantageous, after applying the intermediate varnish coat, to bake at the vulcanizing temperature for a portion of the vulcanizing period and to complete the vulcanization of the rubber by baking at the same temperature after the final coat of varnish has been 45 applied. This procedure somewhat shortens the total time required to complete the process, but it is important that care should be taken on the one hand to avoid overvulcanization of the rubber, and on the other hand that the final coat 50 should receive not less than about one hour's treatment at the full vulcanizing temperature in order to produce the best results and to properly condition the varnish film. However, I do not 55 wish to limit my invention to a process which involves baking the final coat of a two-coat system, since the final coat of varnish may be air-dried or dried at only slightly elevated temperatures. This method is not, however, so desirable 60 because the luster retention of the finish is somewhat reduced when the air-dry procedure is 65 followed.

The two-coat system is preferred to the one-coat system, especially over a rubber coated fabric, because it has greater flexibility and retains its 70 gloss for a longer time. Without limiting myself thereto, I believe this is due to the elastic coat of intermediate varnish acting as a buffer or bridge between the extremely elastic rubber compound and the comparatively inelastic top coat of varnish.

The varnishes herein disclosed, whether air-dried or baked, are useful for finishing fabrics in the production of artificial leather generally and are especially valuable for finishing rubber coated fabrics such as are used on automobile tops, 5 rubber upholstery, etc. These asphalt-oil acid varnishes are superior in compatibility and durability to other varnishes used for this purpose with which I am familiar. In addition to being more compatible, these varnishes do not wrinkle 10 when baked over rubber coated fabrics even when comparatively large amounts of raw China wood oil acids are used. The excellent compatibility of these varnishes makes for good initial luster, freedom from grit, and absence of blue valleys or 15 haze. An outstanding advantage of these varnishes over those heretofore used is their exceptional long retention of luster on outdoor exposure.

With respect to the application of my improved 20 varnishes to fabrics for the production of products having the characteristics of artificial leather, my process has been described in connection with rubber coated fabrics, since these represent the preferred embodiments of the invention, but it is apparent that the finishes disclosed herein may be applied as top coats to flexible sheet material in general, such as cloth and paper fabrics or leather. My improved coating compositions may also be used for the production 30 of artificial leather by finishing coated materials other than rubber coated materials, such as nitro-cellulose coated and linseed oil coated fabrics. The terms "flexible fabric sheeting" and "fabric sheet material", as used herein refer, therefore, 35 to fabrics such as cloth or paper which may be coated with a layer of material such as rubber or pyroxylin; by spraying, spreading, calendering, or by other known methods of application.

As many apparently widely different embodiments of this invention may be made without departing from the spirit and scope thereof, it is to be understood that I do not limit myself to the specific embodiments thereof except as defined in the following claims:

I claim:

1. A coating composition comprising a mixture of free fatty oil acid and asphalt in the proportion of from 20 to 320 parts by weight of the free fatty oil acid to 100 parts by weight of asphalt.
2. A coating composition comprising a mixture of free fatty oil acid and asphalt in the proportion of from 20 to 320 parts by weight of the free fatty oil acid to 100 parts by weight of asphalt, and a varnish drier in an amount sufficient to confer compatibility to said mixture of asphalt and free fatty oil acid.
3. The coating composition set forth in claim 1 in which the free fatty oil acid is drying oil acid.
4. The coating composition set forth in claim 1 in which the free fatty oil acid is linseed oil acid.
5. The coating composition set forth in claim 1 in which the free fatty oil acid is China wood oil fatty acid.
6. The coating composition set forth in claim 1 in which the free fatty oil acid is oleic acid.
7. A process for making artificial leather which comprises applying to fabric sheet material a final coating of a varnish comprising asphalt and free fatty oil acid, and drying said coating, said varnish containing from 20 to 320 pounds by weight of the free fatty oil acid to 100 pounds by weight of asphalt.
8. A process for making artificial leather which comprises applying to rubber sheet material a

final coating of a varnish comprising asphalt and free fatty oil acid, and drying said coating, said varnish containing from 20 to 320 pounds by weight of the free fatty oil acid to 100 pounds by weight of asphalt.

9. A process for making artificial leather which comprises applying to fabric sheet material a final coating of a varnish comprising asphalt, drier, and free fatty oil acid, and baking the resulting product, said varnish containing from 20 to 320 pounds by weight of the free fatty oil acid to 100 pounds by weight of asphalt.

10. As an article of manufacture, a flexible fabric sheeting having a final coat of dried var-

nish comprising asphalt and free fatty oil acid, the free fatty oil acid and asphalt being present in said varnish in the proportion of 20 to 320 pounds by weight of the free fatty oil acid to 100 pounds by weight of asphalt.

11. As an article of manufacture, a rubber coated flexible fabric sheeting having a final coat of dried varnish comprising asphalt and free fatty oil acid, the free fatty oil acid and asphalt being present in said varnish in the proportion of 20 to 320 pounds by weight of the free fatty oil acid to 100 pounds by weight of asphalt.

ALFONSO M. ALVARADO.